

L. WÖHLER.  
CHARGE FOR DETONATOR CASINGS.  
APPLICATION FILED FEB. 26, 1908.

904,289.

Patented Nov. 17, 1908.



Witnesses:  
J. E. Hodges  
H. G. Readdy.

Inventor  
Lothar Wöhler  
by Wright, Brown, Quincy & Key  
Atty's.

# UNITED STATES PATENT OFFICE.

LOTHAR WÖHLER, OF KARLSRUHE, GERMANY.

## CHARGE FOR DETONATOR-CASINGS.

No. 904,289.

Specification of Letters Patent.

Patented Nov. 17, 1908.

Application filed February 25, 1908. Serial No. 417,706.

*To all whom it may concern:*

Be it known that I, LOTHAR WÖHLER, a doctor of philosophy and professor of chemistry in the Karlsruhe Institute of Technology, a subject of the German Emperor, and a resident of 28 Georg Friedrichstrasse, in the city of Karlsruhe, Grand Duchy of Baden, part of the German Empire, have invented certain new and useful Improvements in Charges for Detonator-Casings, of which the following is a specification.

This invention has reference to detonating casings, caps or primers for firing charges of explosive compounds, and it refers in particular to a substitute for the primer or initial igniters heretofore in use.

As a primer, that is to say, a compound which is capable of causing the detonation of all other explosives in contact therewith, when it is ignited itself, only fulminate of mercury has been known and employed heretofore, while other explosive agents, such as iodid of nitrogen, chlorid of nitrogen are not capable of acting as a substitute for this dangerous and expensive agent as a primer, so that heretofore in the majority of cases it has been usual to employ fulminate of mercury either alone or a mixture thereof with chlorate of potash. By making use of the process, described in my prior British patent 21,065, of 1900, the amount of the fulminate employed has already been reduced to only about three tenths of a gram, the charge itself being made up substantially of tri-nitro-toluol and of other explosive agents, but it was not possible to dispense with the use of the fulminate entirely.

I have ascertained, that it is possible to produce the same initial or priming action, as has been produced heretofore by the use of fulminate of mercury, by making use of the salts of the hydrazoic acid or azo-imid or hydrogen-nitrid the formula of which is  $N_2H$ , the said salts having been suggested for use heretofore merely as explosive agents. These salts present the advantage, as compared with fulminate of mercury, that even less than one tenth the amount, required when fulminate of mercury is used, is sufficient as an exploder or primer for igniting other explosives by means of the said salts, and for accomplishing just as complete a de-

tonation of the explosives, contained in the explosive or detonating casing, as it is possible to produce by the use of fulminate of mercury.

The accompanying drawing is a longitudinal sectional view, enlarged from the usual size, of a detonating casing, cap or primer for firing an explosive charge capable of producing the same effect as an ordinary charge for explosive cartridges, usually designated as standard number eight, that is to say cartridges containing two grams of fulminate of mercury. Into the small copper casing *a* of the said cartridge 1 (one) gram of picric acid or of tri-nitro-toluol *b* is placed, and then a quantity of 0.023 (23 thousandths) of a gram of lead hydrazoate *c*, being the lead salt of the hydrazoic acid above referred to, and possessing the formula  $Pb(N_3)_2$ , is placed in a layer upon the charge, and finally a perforated small metal thimble *d* is placed upon the contents, and the entire mass is then compressed in the usual manner.

It is to be understood that I do not limit myself to any particular shape or size of the complete article, nor to its use for any one particular purpose.

What I claim and desire to secure by Letters Patent of the United States, is:—

1. A detonating casing, cap or primer for firing charges of explosive compounds, comprising a cap, containing a heavy metal salt of the hydrazoic acid.

2. A detonating casing, cap or primer for firing charges of explosive compounds, comprising a metal cap, containing superimposed layers of a heavy metal salt of the hydrazoic acid, and an explosive.

3. As an article of manufacture, a detonating cap or primer for firing charges of explosives, comprising a metal cap containing superimposed layers of picric acid and lead hydrazoate.

In witness whereof I have signed my name to this specification in the presence of two subscribing witnesses.

Signed at Mannheim, Germany this 12th day of February 1908.

LOTHAR WÖHLER.

Witnesses:

Jos. H. LEUTE,  
TERESA CATTURANI.